

## UNITED STATES PATENT OFFICE.

EDMOND BOURCART, OF MÜLHAUSEN, GERMANY, ASSIGNOR TO THE FIRM OF "FABRIQUES DES PRODUITS CHIMIQUES DE THANN ET DE MULHOUSE," OF THANN AND MÜLHAUSEN, ALSACE, GERMANY.

## PROCESS OF PRINTING SULFUR DYESTUFFS.

SPECIFICATION forming part of Letters Patent No. 747,295, dated December 15, 1903.

Application filed March 18, 1902. Serial No. 98,799. (No specimens.)

To all whom it may concern:

Be it known that I, EDMOND BOURCART, doctor of philosophy, chemist, a citizen of the Swiss Republic, residing at Mülhausen, Alsace, Germany, have invented a certain new and useful Process of Printing Sulfur Dyestuffs, of which the following is a clear and complete specification.

The so-called "sulfur" dyestuffs, which are formed by the action of alkaline polysulfids on various organic matters, are generally brought on the market mixed with a rather considerable amount of alkaline sulfid. In this state they are not fit for printing, because the sulfid has a destructive action on the copper rollers.

If the free dyestuff is precipitated from its solution, it always retains a large amount of free sulfur, and this free sulfur forms again alkaline sulfid when the color is mixed with alkali. If the sulfur is entirely eliminated by several extractions with carbon disulfid, the coloring-matter is no more able to be printed with caustic alkali alone. Addition of reducing organic bodies—for instance, glucose, glycerin, &c.—has not given satisfactory results.

The following process is in every case a successful one.

30 The commercial coloring-matter is precipitated from its solution in alkaline sulfid by means of an acid, and the precipitate is washed until the acid reaction has disappeared. It contains then more or less of free sulfur. 35 This precipitate, as it is or after spontaneous oxidation, mixed with a thickening, a certain amount of an alkaline carbonate, (neutral carbonate or bicarbonate,) and at least one reducing agent—as, for instance, sodium 40 thiosulfate, sulfite, formate or xanthate, sulfur, glucose, &c.—is ready for printing and does no more attack the copper rollers.

The sulfur and the other reducing agents act only when the cloth is steamed. Therefore 45 the printing-color is stable and may be kept for a certain time, whereas the color reduced before printing oxidizes itself rapidly in the presence of air, a fact which contributes to make disadvantageous the processes known

hitherto. The alkaline carbonate or bicarbonate and the free sulfur yield on steaming alkaline sulfid, which serves to fix the coloring-matter, and in presence of a reducing agent this fixation is more rapid. The patterns printed in this way resist completely to washing and soaping without staining the white ground.

All the sulfur dyestuffs tried hitherto—for instance, Bayer's katigene, Cassella's immedi-al, the kryogen of the Badische Anilin und Soda Fabrik, the pyrogene or sulfogene of the Society of Chemical Industry, Leonhardt's pyrol, &c.—may be printed in this way.

As an illustration of my process the following directions may be given:

I. Ten parts pure immedi-al blue B extra in paste, fifty parts thickening, ten parts sodium bicarbonate, five parts sodium thiosulfate, twenty-five parts water.

II. Thirty parts of pyrogene black G in paste, fifty parts thickening, ten parts sodium bicarbonate, five parts glucose, five parts water.

III. Thirty parts kryogen brown in paste form, fifty parts thickening, ten parts sodium bicarbonate, five parts sodium formate, five parts water.

IV. Thirty parts pyrol black B in paste form, fifty parts thickening, five parts sodium sulfite, ( $Na_2SO_3$ ), ten parts sodium bicarbon- ate, five parts water.

V. Twenty-five parts katigene green 2B in paste form, fifty parts thickening, ten parts sodium bicarbonate, three parts zinc sulfid, ( $ZnS$ ), twelve parts water.

VI. Twenty parts katigene indigo paste, ten parts sodium bicarbonate, five parts sodium xanthate, sixty-five parts thickening.

Metallic carbonates or sulfids may be added to these colors in order to change the shade and increase the solidity. If the colors are less thickened in order to keep them more fluid, they may be used for padding and produce plain pattern by steaming. The printing as well as the padding colors may be reserved by acid discharges or by soluble salts of such metals as form insoluble carbonates printed before steaming.

2  
What I claim is—

1. The herein-described process of printing with a sulfur dyestuff which has been precipitated from its solution and which contains free sulfur but no alkaline sulfid, said process consisting in first mixing said precipitate with a thickening material, water, an alkaline bicarbonate and at least one reducing agent at the ordinary temperature, in order to produce a printing-paste containing the sulfur dyestuff in a non-reduced state, then printing and finally steaming the fabric after printing in order to form the alkaline sulfid necessary to fix the dyestuff.
- 15 2. The herein-described process of printing with a sulfur dyestuff which has been precipitated from its solution and which con-

tains free sulfur but no alkaline sulfid, said process consisting in first mixing said precipitate with a thickening material, water, 20 an alkaline bicarbonate and at least one reducing agent at the ordinary temperature, in order to produce a printing-paste containing the sulfur dyestuff in a non-reduced state, then printing and finally steaming the fabric 25 after printing in order to form the alkaline sulfid necessary to fix the dyestuff.

In witness whereof I have hereunto signed my name, this 6th day of March, 1902, in the presence of two subscribing witnesses.

EDMOND BOURCART.

Witnesses:

CHARLES MENNIER-DAUPP,  
AMAND RITTER.